

# United States Patent Office

2,925,351

Patented Feb. 16, 1960

SEARCHED, SERIALIZED, INDEXED, AND MICROFILMED

1

2,925,351

## PORCELAIN ENAMELS FOR LIGHT METALS

Donald M. Judd, Cleveland, Ohio, assignor to Ferro Corporation, Cleveland, Ohio, a corporation of Ohio

No Drawing. Application August 9, 1957

Serial No. 677,231

7 Claims. (Cl. 106—48)

This invention relates as indicated to porcelain enamels for light metals and has particular reference to resistant protective and decorative porcelain enamels for aluminum and aluminum alloys.

Numerous attempts have been made in the past to protect and/or decorate aluminum and its alloys. However, these prior art porcelain enamels are all what are known as lead bearing and contain the basic toxic effects inherent in all lead containing porcelain enamels. The temperatures at which porcelain enameling of aluminum and its alloys would be permissible, are much lower than those temperatures used to porcelain enamel cast iron and steel. Thus lead has been used to produce porcelain enamels having a maturing temperature compatible with aluminum.

I have now discovered certain new and improved high alkali containing porcelain enamel compositions which are lead-free, have a maturing temperature compatible with the melting temperature of aluminum and which may be satisfactorily applied to surfaces of aluminum and its alloys whether the metal is rolled, drawn or cast and which porcelain enamels provide hard, smooth, glossy coatings.

It is an object of this invention to provide new and improved porcelain enamels for application to aluminum and its alloys which are lead-free.

It is another object of this invention to produce high alkali containing porcelain enamels which are lead-free and which may be applied to aluminum and its alloys at temperatures so low that the application of the porcelain enamel to the metal need not damage any special metallurgical properties of the metal.

It is a further object of this invention to provide porcelain enamel compositions which are lead-free, fluorine-free and which can be fused to aluminum and its alloys at a temperature between 900° F. and 1050° F. and which will furnish a durable smooth glossy coating.

Other objects will become apparent as the description proceeds.

To the accomplishment of the foregoing and related ends, said invention then comprises the features herein-after fully described and particularly pointed out in the claims, the following description setting forth in detail certain illustrative embodiments of the invention, these being indicative, however, of but a few of the various ways in which the principle of the invention may be employed.

Broadly stated this invention comprises a lead-free porcelain enamel having a firing temperature of between 900° F. and 1050° F. which consists essentially of the following constituents calculated as weight percentages:

|          | Percent |
|----------|---------|
| $R_2O_1$ | 21-35   |
| $R_2O_3$ | 2-5     |
| $R_2O_5$ | 11-21   |
| $RO_2$   | 44-50   |

2

where  $R_2O$  represents the oxides of Na, K and Li;  $R_2O_3$  represents the oxide of B;  $R_2O_5$  represents the oxides of P and Sb; and  $RO_2$  represents the oxides of Si and Ti.

From the foregoing broadly stated paragraph it will be readily seen that the compositions of the present invention are radically different from the aluminum porcelain enamels known to those skilled in the art. In contrast with prior art compositions the present porcelain enamels do not contain lead, fluorine and/or cadmium and additionally it will be seen that the present enamels do not contain the RO group which comprises the oxides of the elements Mg, Ca, Zn, Sr and/or Ba. Still further the present compositions will be found to be extremely low in  $B_2O_3$  (2%-5%) and to be free of  $Al_2O_3$ .

I have found that low melting lead-free porcelain enamels having a coefficient of expansion suitable for application to aluminum or aluminum base alloys can be made if certain basic concepts are followed. First, the alkali oxide content of the porcelain enamel must be high, from 21% to 35% of the total composition, in order to obtain a frit which will have a sufficiently low firing temperature. Second, the  $B_2O_3$  must be low, from 2%-5% of the total composition, in order to obtain a frit having a coefficient of expansion sufficiently high to insure good bond with the aluminum work piece. Third, the  $SiO_2$  and  $TiO_2$  must be from 44% to 50% of the total composition in order to obtain a glass having good chemical and physical properties, such as, acid resistance, smooth surface and durability.

The constituents of my novel porcelain enamels can be expressed as weight percentages within the following ranges:

|           | Percent   |
|-----------|-----------|
| $B_2O_3$  | 2.0-5.0   |
| $Na_2O$   | 9.5-16.0  |
| $K_2O$    | 10.0-18.0 |
| $Li_2O$   | 2.0-6.0   |
| $TiO_2$   | 20.0-27.0 |
| $P_2O_5$  | 1.0-3.0   |
| $Sb_2O_5$ | 10.0-18.0 |
| $SiO_2$   | 17.0-29.0 |

It will be observed that not only is there an absence of lead and the RO (alkaline earth) elements but the proportion of boric oxide does not exceed 5.0% and there is no aluminum oxide present. On the other hand, the  $R_2O$  (alkali oxides) percentages are high.

The foregoing constituents provide porcelain enamels having all the necessary chemical and physical properties for application to aluminum and aluminum base alloys. The high alkali metal oxides provides the necessary fluidity to the porcelain enamel during the firing operation. The boric oxide is a factor in controlling the gloss of the fired porcelain enamel. The  $P_2O_5$  and  $Sb_2O_5$  are important in controlling during firing, the reaction between the porcelain enamel and the aluminum work piece, they also give good tearing and spalling resistance properties to the porcelain enamel and additionally contribute to the glossy surface of the fired piece. The  $SiO_2$  is the glass former and the  $TiO_2$  gives the porcelain enamel chemical durability or what is known as acid resistance. Additionally the  $TiO_2$  serves to give refractoriness to the composition.

In the event it is found desirable to adjust the amounts of the various ingredients of the present porcelain enamels for best results, it will be found expedient to bear the following factors in mind:

(1) The ratio of the weight percent of  $SiO_2$  to the weight percent of  $TiO_2$  should be kept between 0.8 and 1.3;

(2) The ratio of the weight percent of  $Sb_2O_5$  to the weight percent of  $B_2O_3$  should be kept between 1.2 and 8.5; and

(3) The  $Li_2O$  should be about 9-18% of the total alkali oxide content, the  $Na_2O$  about 30-50% of the total alkali oxide content and the  $K_2O$  about 32-56% of the total alkali oxide content.

The ingredients used in making up a batch composition may take the form of oxides, carbonates, nitrates, silicates, etc. As for example, dehydrated borax, soda ash, potassium carbonate, titanium dioxide, monoammonium phosphate, lithium carbonate, sodium antimonate and powdered quartz are typical of raw materials used to make the present compositions.

It will be understood that other suitable raw batch ingredients can be used in making the frits of the present invention. Thus, soda nitrate can be substituted for soda ash, antimony oxide may be substituted for sodium antimonate, etc., it being understood that the amounts of such altered raw materials are calculated to yield the desired frit composition.

In the preparation of these frits the raw materials are weighed and thoroughly mixed. The mixed batch is then smelted either in a batch type or a continuous type smelter and smelted to a homogeneous glass. Smelting temperatures may vary within wide limits, however, 2100° F.-2300° F. is a particularly suitable range. The molten glass is then fritted with air or water by any of the well known methods.

The frit is then wet ground or dry ground, with suitable mill addition agents in a ball mill or other mill to a predetermined fineness. The compositions of our invention produce substantially white semi-opaque porcelain enamels. If an opaque or colored porcelain enamel is desired it is convenient, during the grinding operation, to add the desired opacifying agents (such as  $TiO_2$ ) or coloring pigments in addition to the normally used suspending agents, bonding agents, etc.

The milled frit which has been suspended in a suitable vehicle may be applied to the aluminum work piece by any of the well known procedures of spraying, dipping, slushing, brushing, etc.

After application of the powdered frit to the aluminum work piece it is fired for several minutes in a suitable furnace in order to fuse the frit onto the surface of the work piece. The firing temperatures are not critical since the compositions of my invention mature at from 900° F. to 1050° F. The temperature used in melting or fusing the frit onto the work piece depends to some extent on the particular aluminum alloy being coated and on the particular porcelain enamel composition selected.

Other modes of applying the principle of the invention may be employed, change being made as regards the details described, provided the features stated in any of the following claims or the equivalent of such be employed.

I, therefore, particularly point out and distinctly claim as my invention:

1. A lead-free, alumina-free porcelain enamel having a firing temperature range of between 900° F. and 1050° F. which consists essentially of the following constituents calculated as weight percentages:

|          | Percent |
|----------|---------|
| $R_2O$   | 21-35   |
| $R_2O_3$ | 2-5     |
| $R_2O_5$ | 11-21   |
| $RO_2$   | 44-50   |

where  $R_2O$  represents the oxides Na, K and Li;  $R_2O_3$  represents the oxide of B;  $R_2O_5$  represents the oxides of P and Sb; and  $RO_2$  represents the oxides of Si and Ti, the summation of the weight percentages of  $R_2O$ ,  $R_2O_3$ ,  $R_2O_5$ , and  $RO_2$  ingredients equalling 100%.

2. A lead-free, alumina-free porcelain enamel having a firing temperature range of between 900° F. and 1050° F.

which consists essentially of the following constituents calculated as weight percentages:

|          | Percent |
|----------|---------|
| $R_2O$   | 21-35   |
| $R_2O_3$ | 2-5     |
| $R_2O_5$ | 11-21   |
| $RO_2$   | 44-50   |

where  $R_2O$  represents the oxides Na, K and Li;  $R_2O_3$  represents the oxide of B;  $R_2O_5$  represents the oxides of P and Sb; and  $RO_2$  represents the oxides of Si and Ti, wherein the  $Li_2O$  is about 9-18% of the total  $R_2O$  content, the  $Na_2O$  is about 30-50% of the total  $R_2O$  content and the  $K_2O$  is about 32-56% of the total  $R_2O$  content, the summation of the weight percentages of  $R_2O$ ,  $R_2O_3$ ,  $R_2O_5$ , and  $RO_2$  ingredients equalling 100%.

3. A lead-free, alumina-free porcelain enamel having a firing temperature range of between 900° F. and 1050° F. which consists essentially of the following constituents calculated as weight percentages:

|          | Percent |
|----------|---------|
| $R_2O$   | 21-35   |
| $R_2O_3$ | 2-5     |
| $R_2O_5$ | 11-21   |
| $RO_2$   | 44-50   |

where  $R_2O$  represents the oxides Na, K and Li;  $R_2O_3$  represents the oxide of B;  $R_2O_5$  represents the oxides of P and Sb; and  $RO_2$  represents the oxides of Si and Ti, wherein the ratio of the weight percent of  $Sb_2O_5$  to the weight percent of  $B_2O_3$  is between 1.2 and 8.5, the summation of the weight percentages of  $R_2O$ ,  $R_2O_3$ ,  $R_2O_5$ , and  $RO_2$  ingredients equalling 100%.

4. A lead-free, alumina-free porcelain enamel having a firing temperature range of between 900° F. and 1050° F. which consists essentially of the following constituents calculated as weight percentages:

|          | Percent |
|----------|---------|
| $R_2O$   | 21-35   |
| $R_2O_3$ | 2-5     |
| $R_2O_5$ | 11-21   |
| $RO_2$   | 44-50   |

where  $R_2O$  represents the oxides Na, K and Li;  $R_2O_3$  represents the oxide of B;  $R_2O_5$  represents the oxides of P and Sb; and  $RO_2$  represents the oxides of Si and Ti, wherein the ratio of the weight percent of  $SiO_2$  to the weight percent of  $TiO_2$  is between 0.8 and 1.3, the summation of the weight percentages of  $R_2O$ ,  $R_2O_3$ ,  $R_2O_5$ , and  $RO_2$  ingredients equalling 100%.

5. A lead-free, alumina-free porcelain enamel having a firing temperature range of between 900° F. and 1050° F. which consists essentially of the following constituents calculated as weight percentages and totalling 100 weight percent:

|           | Percent   |
|-----------|-----------|
| $B_2O_3$  | 2.0-5.0   |
| $Na_2O$   | 9.5-16.0  |
| $K_2O$    | 10.0-18.0 |
| $Li_2O$   | 2.0-6.0   |
| $TiO_2$   | 20.0-27.0 |
| $P_2O_5$  | 1.0-3.0   |
| $Sb_2O_5$ | 10.0-18.0 |
| $SiO_2$   | 17.0-29.0 |

wherein the ratio of the weight percent of  $SiO_2$  to the weight percent of  $TiO_2$  is between 0.8 and 1.3, the ratio of the weight percent of  $Sb_2O_5$  to the weight percent of  $B_2O_3$  is between 1.2 and 8.5 and the  $Li_2O$  is about 9-18% of the total alkali oxide ( $Li_2O+Na_2O+K_2O$ ) content, the  $Na_2O$  is about 30-50% of the total alkali oxide ( $Li_2O+Na_2O+K_2O$ ) content and the  $K_2O$  is about 32-56% of the total alkali oxide ( $Li_2O+Na_2O+K_2O$ ) content, said total alkali oxide ( $Li_2O+Na_2O+K_2O$ ) content being from 21-35% of the total composition.

6. A lead-free, alumina-free porcelain enamel having a

firing temperature range of between 900° F. and 1050° F. which consists essentially of the following constituents calculated as weight percentages and totalling 100 weight percent:

|                                | Percent   |
|--------------------------------|-----------|
| B <sub>2</sub> O <sub>3</sub>  | 2.0- 5.0  |
| Na <sub>2</sub> O              | 9.5-16.0  |
| K <sub>2</sub> O               | 10.0-18.0 |
| Li <sub>2</sub> O              | 2.0- 6.0  |
| TiO <sub>2</sub>               | 20.0-27.0 |
| P <sub>2</sub> O <sub>5</sub>  | 1.0- 3.0  |
| Sb <sub>2</sub> O <sub>5</sub> | 10.0-18.0 |
| SiO <sub>2</sub>               | 17.0-29.0 |

wherein the ratio of the weight percent of SiO<sub>2</sub> to the weight percent of TiO<sub>2</sub> is between 0.8 and 1.3, the ratio of the weight percent of Sb<sub>2</sub>O<sub>5</sub> to the weight percent of B<sub>2</sub>O<sub>3</sub> is between 1.2 and 8.5 and the Li<sub>2</sub>O is about 9-18% of the total alkali oxide (Li<sub>2</sub>O+Na<sub>2</sub>O+K<sub>2</sub>O) content, the

5

10

Na<sub>2</sub>O is about 30-50% of the total alkali oxide (Li<sub>2</sub>O+Na<sub>2</sub>O+K<sub>2</sub>O) content and the K<sub>2</sub>O is about 32-56% of the total alkali oxide (Li<sub>2</sub>O+Na<sub>2</sub>O+K<sub>2</sub>O) content, said total alkali oxide (Li<sub>2</sub>O+Na<sub>2</sub>O+K<sub>2</sub>O) content being from 21-35% of the total composition, and said SiO<sub>2</sub>+TiO<sub>2</sub> comprising from 44%-50% of the total composition.

7. An article of manufacture comprising an aluminum work piece containing as a protective and decorative coating thereon the procelain enamel of claim 6.

References Cited in the file of this patent

UNITED STATES PATENTS

|           |                        |               |
|-----------|------------------------|---------------|
| 2,492,523 | Coffeen et al. -----   | Dec. 27, 1949 |
| 2,537,956 | Baldwin -----          | Jan. 16, 1951 |
| 2,662,020 | Schofield et al. ----- | Dec. 8, 1953  |
| 2,800,414 | Stradley et al. -----  | July 23, 1957 |
| 2,827,393 | Kadisch et al. -----   | Mar. 18, 1958 |